# EUROPEAN PATENT SPECIFICATION

(11) **EP 2 781 629 B1**
(45) Date of publication and mention of the grant of the patent: **14.09.2016**
(21) Application number: 14160514.7
(22) Date of filing: 18.03.2014
(51) Int. Cl.: C25D 3/62

(54) **Solution for the electrodeposition of a gold alloy and the alloy derived therefrom**
Lösung zur Elektrotauchbeschichtung einer Goldlegierung sowie daraus erhaltene Legierung
Solution pour l'électrodéposition d'un alliage d'or et alliage en dérivant

(30) Priority: 18.03.2013 IT FI20130057
(43) Date of publication of application: 24.09.2014
(73) Proprietor: Bluclad S.R.L., 59100 Prato (IT)
(72) Inventor: Carlan, Fabrizio, 59100 PRATO (IT); Paoli, Daniele, 59100 PRATO (IT); Cavaciocchi, Lorenzo, 50058 SIGNA (IT); Banchelli, Elena, 59100 PRATO (IT); Luconi, Leandro, 59100 PRATO (IT); Canelli, Danilo Vincenzo, 59100 MONTALE (IT)
(74) Representative: Valenza, Silvia

(56) References cited:
- WO-A1-02/068728
- GB-A- 1 325 352
- GB-A- 2 306 508
- GB-A- 2 323 853
- US-A- 3 475 292
- US-A- 3 502 548
- US-A- 3 904 493
- US-A- 3 990 954
- US-A- 4 075 065

## Description

FIELD OF THE INVENTION

The present invention relates to the field of solutions for electrodeposition of metal alloys and derived alloys; in particular, it relates to a solution for the electrodeposition of a gold alloy and to the alloy derived therefrom having defined colour coordinates in the range of (L: 65-75; a: 6-9; b: 10-20).

### PRIOR ART

The metal alloys obtained by electrodeposition are widely used in various production sectors, both for the physical qualities thereof and for the specific aesthetic nature thereof.

Coloured alloys, obtained by the electrodeposition of metals, both individually and alloyed together, are found to be of interest for this second purpose; these alloys are put to practical use in various fields: furniture, clothing, jewellery, and in general any sectors requiring articles having specific aesthetic properties.

Coloured Gold alloys are found to be among the most used since they make it possible to obtain a vast range of colours and shades depending on the formulation used and the working conditions applied to obtain them.

Thus far, with galvanic gilding baths, it is possible to obtain the entire range of colours and shades of the colours white, yellow, pink and even green; however, brown colours are difficult to obtain under simple conditions and using chemically stable solutions.

US 4 075 065 A discloses an acidic electroplating bath comprising 0.1-50 g/ I alkali gold cyanide, 5-250 g/l zirconium oxychloride or vanadyl sulphate, 0.01-15 g/ I metallic hardener, selected from Fe, Co or Ru. The bath is used for plating a Au-Fe-V alloy layer.

GB 2 306 508 A discloses a gold alloy (Au-Fe-Zr) electrodeposit containing 1.25 to 1.55 wt% Fe, 1 to 2 ppm Zr and 97.7 to 98.2 wt% Au, and which has a pale yellow colour less than 3N.

GB 2 323 853 A discloses a gold alloy (Au-Fe-Ti) electrodeposit containing 1.25 to 1.55 wt% Fe, 1 to 2 ppm Ti and 97.7 to 98.2 wt % Au, and which has a pale yellow colour less than 3N.

There is therefore an interest in the formulation of chemically stable galvanic baths which are easy to manage and handle and can be used for the electrodeposition of brown gold alloys having colour coordinates in the range of: (L: 65-75; a: 6-9; b: 10-20) and having a shiny and coherent deposit.

### SUMMARY OF THE INVENTION

The present invention solves the above problems by way of an aqueous solution for the electrodeposition of a Gold alloy; said solution comprising a Gold (Au) salt, an Iron (Fe) salt and a Vanadium (V) salt, and optionally one or more salts of other metals suitably selected among the Cobalt (Co), Palladium (Pd), Ruthenium (Ru) salts, for modulating the end colour shades; and optionally further comprising small amounts of one of more Tellurium (Te), Gallium (Ga) or Bismuth (Bi) salts, as sparkling aids and grain refiners.

The alloy derived from the aforementioned solution has colour coordinates in the range of: (L: 65-75; a: 6-9; b: 10-20).

The invention thus relates to a gold alloy having colour coordinates in the range of: (L: 65-75; a: 6-9; b: 10-20), said alloy, which can be obtained from the aforementioned solution, having the following percentage composition by weight:
- Au 86-91 %;
- Fe 6-8%
- V 4-6%
- Co, Pd, Ru or mixtures thereof 0-0.5%. Te, Ga, Bi or mixtures thereof are not alloyed, but merely serve as sparkling aids.

The invention also relates to a method for the electrodeposition of a gold alloy as disclosed above using the aforementioned solution.

### DETAILED DESCRIPTION OF THE INVENTION

For the purposes of the present invention, a solution for electrodeposition is a galvanic bath and the solvent used is water.

The solution preferably contains a suitable buffer system, one or more complexing agents which guarantee stability of the metals in solution in addition to modulating the alloying thereof, and a surfactant which also acts as a sparkling aid.

The Gold salt may be Gold chloride, Gold sulphite, potassium Dicyanoaurate, potassium Tetracyanoaurate, ammonium Cyanoaurate or a combination thereof.

The concentration of Gold as a metal is in the range of 0.5 to 3 g/L, preferably from 0.7 to 1.8 g/L, the most suitable concentration for obtaining the desired triplet of colour coordinates in the range of interest (L: 65-75; a: 6-9; b:10-20) being selected from time to time.

The metals which are alloyed with the Gold are primarily Iron and Vanadium, introduced into the solution in the form of the most common salts thereof, such as, for Iron, by way of non-limiting example, Iron sulphate, Iron carbonate, Iron acetate, Iron citrate and Iron chloride, depending on the selected buffer system and on the stability of the selected salt in the environment of the solution, and for Vanadium, by way of non-limiting example, Vanadium Oxychloride, Vanadium Oxytriethoxide, Vanadium Oxytripropoxide, Vanadium Oxyfluoride, Vanadium Oxide, Sodium Vanadium Oxide, Vanadium halide.

The concentrations of the aforementioned metals are in the range of 0.2 g/L to 1 g/L, the most suitable concentration of each of these for obtaining the desired triplet of colour coordinates in the range of interest (L: 65-75; a: 6-9; b:10-20) being selected from time to time.

The pH is maintained in a range between 7 and 10. These metals are used so as to obtain a reduction in the values of the colour coordinates a and b with respect to the typical values for a 24 kt Gold deposits (L = 84-85; a = 6-8; b = 30-31); the amounts added for each individual metal bring about a corresponding effect on these coordinates in relation to the concentration. The other metals which may be introduced into the solution as salts for modulating the colour shades are Cobalt, Palladium, Ruthenium and mixtures thereof, these also being introduced into the solution in the form of the most common salts thereof, such as, by way of non-limiting example, sulphate, carbonate, acetate, citrate and chloride, depending on the selected buffer system and on the stability of the selected salt in the environment of the solution.

The concentrations of each of these metals are in the range of 0.005 to 0.5 g/L, the most suitable concentration of each of these for obtaining the desired triplet of colour coordinates in the range of interest (L: 65-75; a: 6-9; b:10-20) being selected from time to time.

These metals are used so as to obtain a modulation of the values of the colour coordinates a and b with respect to the typical values for a 24 kt Gold deposits (L = 84-85; a = 6-8; b = 30-31); the amounts added for each individual metal bring about a corresponding effect on these coordinates in relation to the concentration. In particular, it has been found that:
- Ruthenium reduces the L coordinate;
- Palladium and Cobalt increase the L coordinate;

It has further been found that Tellurium, Gallium and Bismuth or combinations thereof improve the homogeneity of the colour of the deposit and refine the grain of the deposit: they are introduced into the solution in the form of the soluble salts thereof or stable complexes thereof in the working conditions of the solution, in amounts for each metal in the range of 0.005 - 0.015 g/L as a metal.

The pH of the solution is not a critical parameter apart from for the stability in solution of the selected metals, and is between 7 and 10, preferably between 7.5 and 9.5, and is regulated using sodium or potassium hydroxide or using inorganic acids such as, by way of non-limiting example, sulphuric acid, phosphoric acid, formic acid.

In working conditions, the pH is kept stable by way of a buffer system selected among the acid/salt pairs of acids such as gluconic, oxalic, citric, tartaric, malonic, malic, phosphoric and sulphamic acid *inter alia,* which serve as complexing agents for the metals in solution, promoting the stability thereof, in addition to guaranteeing pH stability.

The salts of the aforementioned acids may be sodium or potassium salts or salts of other alkali and alkaline earth metals which are soluble in the conditions of the solution.

The concentrations of the acids and the salts thereof are in the range of 30 g/L to 170 g/L, more favourable of 50 g/L to 130 g/L.

It is also favourable to introduce one or more complexing agents into the solution, in concentrations of between 20 and 50 g/L, such as ethylenediaminetetraacetic acid, etidronic acid, nitrilotriacetic acid, ethylenediamine tetra methylenephosphonic acid, nitrilotrismethylenediphosphonic acid, in the form of the free acid or in the form of a salt.

The selection of the form of the complexing agent, the concentration and the composition of the eventual mixture is determined by the colour coordinates in the range of interest (L: 65-75; a: 6-9; b: 10-20) which it is desired to obtain.

The surfactant is selected from the sodium salts of the alkylsulphonates and alkylphosphonates which are soluble and stable at the working pH of the invention, and is used in an amount of no more than 1 g/L, introduced as a pre-diluted aqueous solution to avoid solubility problems.

The temperature and current density applied to the solution are parameters which influence the colour coordinates, and therefore have to be applied within particular intervals and modulated on the basis of the colour coordinates which it is desired to obtain in the range of interest (L: 65-75; a: 6-9; b: 10-20).

The preferred working temperature of the solution is in the range of 35 to 45°C; an increase in temperature leads to an increase in Gold in the deposit and thus raises the a and b coordinates.

The preferred current density is in the range of 0.5 A/dm² to 3 A/dm³; an increase in applied current density initially leads to an alteration to the colour and subsequently to the appearance of burns and localised inhomogeneities of the deposit.

The duration of application of the current does not influence the colour, but in relation to a colouring bath the deposition times may typically be up to 2 minutes of application.

A better understanding of the invention may be gained from the following practical examples.

### EXPERIMENTAL PART

### Example No. 1

The following aqueous solution was prepared:
Citric Acid 30 g/L
Potassium Citrate 90 g/L
HEDP tetrasodium 7 g/L
Gold 1 g/L introduced as Potassium Dicyanoaurate
Iron 0.6 g/L introduced as Iron Citrate
Vanadium 0.6 g/L introduced as Vanadium Oxychloride
Tellurium 0.005 g/L introduced as Tellurium Oxide
Sodium Lauryl Ether 0.1 mL/L of the 10% w/v solution

A sheet of copper of size 10 × 10 cm, on which a layer of 24 kt Gold having colour coordinates (L = 84.8; a = 7.7; b = 30.2) had previously been deposited, was plated with the above-disclosed solution in the laboratory under the following working conditions:
pH 8
45 °C
0.8 A/dm²
1 minute

The sheet was then rinsed in demineralised water and dried in an oven at 85°C for 30 minutes, then left to cool to room temperature.

The colour coordinates obtained were measured and found to be: L: 72; a: 7.3; b: 15.2

From electron microscope analysis, the alloy was found to have the following average % composition by weight:
Au 89.4 %
Fe 6.65 %
V 3.95 %
Te did not alloy.

## Claims

1. A gold alloy having color coordinates in the range: L: 65-75; a: 6-9; b: 10-20 and having the following percentage composition by weight:
| | |
|---|---|
| Au | 86-91%; |
| Fe | 6-8% |
| V | 4-6% |
| Co, Pd, Ru or mixtures thereof | 0-0.5% |

2. A method for the electrodeposition of a gold alloy according to claim 1; said method comprising the use of an aqueous solution comprising a Gold (Au) salt, an Iron (Fe) salt and a Vanadium (V) salt, and optionally one or more salts of other metals suitably selected among the Cobalt (Co), Palladium (Pd), Ruthenium (Ru) salts, for modulating the end color shades; and optionally further comprising small amounts of one of more Tellurium (Te), Gallium (Ga) or Bismuth (Bi) salts, as sparkling aids and grain refiners, wherein Gold as a metal is in the range between 0.5 and 3 g/L, wherein Fe and V as metals are provided in concentrations in the range between 0.2 and 1 g/L, respectively, and having a buffered pH in the range between 7 and 10.

3. Method according to claim 2, wherein Gold as a metal is in the range between 0.7 and 1.8 g/L.

4. Method according to claim 2, wherein Fe and V as metals are provided in concentrations of 0.6 g/L, respectively.

5. Method according to claim 2, wherein Co, Pd and Ru, if provided, are each provided in concentrations in the range between 0.005 and 0.5 g/L, wherein the concentrations are referred to the metal in solution.

6. Method according to claim 2, wherein Te, Ga, Bi or combinations thereof are introduced in the solution in the form of soluble salts thereof or stable complexes thereof in the working conditions of the solution, in amounts for each metal in the range between 0.005 and 0.015 g/L as a metal.

7. Method according to any one of claims 2-6, having a buffered pH in the range between 7.5 and 9.5

8. Method according to any one of claims 2-7, comprising one or more complexing agents in concentrations in the range between 20 and 50 g/L.

9. Method according to any one of the preceding claims, wherein a surfactant agent is provided in amounts of no more than 1 g/L.

10. An aqueous solution for the electrodeposition of a gold alloy according to claim 1; said solution comprising a Gold (Au) salt, an Iron (Fe) salt and a Vanadium (V) salt, and optionally one or more salts of other metals suitably selected among the Cobalt (Co), Palladium (Pd), Ruthenium (Ru) salts, for modulating the end color shades; and optionally further comprising small amounts of one of more Tellurium (Te), Gallium (Ga) or Bismuth (Bi) salts, as sparkling aids and grain refiners, wherein Gold as a metal is in the range between 0.5 and 3 g/L, wherein Fe and V as metals are provided in concentrations in the range between 0.2 and 1 g/L, respectively, and having a buffered pH in the range between 7 and 10.

## Patentansprüche

1. Goldlegierung mit Farbkoordinaten im Bereich: L: 65-75; a: 6-9; b: 10-20 und mit der folgenden Zusammensetzung in Gewichtsprozent:
| | |
|---|---|
| Au | 86-91 %; |
| Fe | 6-8 % |
| V | 4-6 % |
| Co, Pd, Ru oder Mischungen davon | 0-0,5 %. |

2. Verfahren zur elektrochemischen Abscheidung einer Goldlegierung gemäß Anspruch 1, wobei genanntes Verfahren die Verwendung einer wässrigen Lösung umfasst, die ein Gold(Au)-Salz, ein Eisen(Fe)-Salz und ein Vanadium(V)-Salz und gegebenenfalls ein oder mehrere Salze anderer Metalle umfasst, die auf geeignete Weise ausgewählt sind aus Cobalt(Co)-, Palladium(Pd)-, Ruthenium(Ru)-Salzen, zum Modulieren der Endfarbnuancen, und gegebenenfalls des Weiteren umfassend geringe Menge n von einem von mehreren Tellur(Te)-, Gallium(Ga)- oder Bismut(Bi)-Salzen als Sprudelhilfen und Kornfeinungsmittel, wobei Gold als ein Metall im Bereich zwischen 0,5 und 3 g/l vorliegt, wobei Fe und V als Metalle in Konzentrationen im Bereich von 0,2 bzw. 1 g/l vorliegen und mit einem gepufferten pH-Wert im Bereich zwischen 7 und 10.

3. Verfahren gemäß Anspruch 2, wobei Gold als Metall im Bereich zwischen 0,7 und 1,8 g/l vorliegt.

4. Verfahren gemäß Anspruch 2, wobei Fe und V als Metalle jeweils in Konzentrationen von 0,6 g/l bereitgestellt werden.

5. Verfahren gemäß Anspruch 2, wobei Co, Pd und Ru, sofern bereitgestellt, jeweils in Konzentrationen im Bereich zwischen 0,005 und 0,5 g/l bereitgestellt werden, wobei die Konzentrationen sich auf das Metall in Lösung beziehen.

6. Verfahren gemäß Anspruch 2, wobei Te, Ga, Bi oder Kombinationen davon in Form von löslichen Salzen davon oder von unter den Arbeitsbedingungen der Lösung stabilen Komplexen davon in die Lösung eingeführt werden, wobei die Mengen für jedes Metall im Bereich zwischen 0,005 und 0,015 g/l als ein Metall liegen.

7. Verfahren gemäß einem der Ansprüche 2 bis 6 mit einem gepufferten pH-Wert im Bereich zwischen 7,5 und 9,5.

8. Verfahren gemäß einem der Ansprüche 2 bis 7, umfassend ein oder mehrere Komplexierungsmittel in Konzentrationen im Bereich zwischen 20 und 50 g/l.

9. Verfahren gemäß jedem der vorhergehenden Ansprüche, wobei ein Tensid in Mengen von höchstens 1 g/l bereitgestellt wird.

10. Wässrige Lösung zur elektrochemischen Abscheidung einer Goldlegierung gemäß Anspruch 1, wobei genannte Lösung ein Gold(Au)-Salz, ein Eisen(Fe)-Salz und ein Vanadium(V)-Salz und gegebenenfalls ein oder mehrere Salze anderer Metalle umfasst, die auf geeignete Weise ausgewählt sind aus Cobalt(Co)-, Palladium(Pd)-, Ruthenium(Ru)-Salzen, zum Modulieren der Endfarbnuancen, und gegebenenfalls des Weiteren umfassend geringe Mengen von einem von mehreren Tellur(Te)-, Gallium(Ga)- oder Bismut(Bi)-Salzen als Sprudelhilfen und Kornfeinungsmittel, wobei Gold als ein Metall im Bereich zwischen 0,5 und 3 g/l vorliegt, wobei Fe und V als Metalle in Konzentrationen im Bereich von 0,2 bzw. 1 g/l vorliegen und mit einem gepufferten pH-Wert im Bereich zwischen 7 und 10.

## Revendications

1. Alliage d'or ayant des coordonnés de couleur dans la plage : L : 65 à 75 ; a : 6 à 9 ; b : 10 à 20 et ayant la composition en pourcentage en poids suivante :
| | |
|---|---|
| Au | 86 à 91 % ; |
| Fe | 6 à 8 % ; |
| V | 4 à 6 % ; |
| Co, Pd, Ru ou mélanges de ceux-ci 0 à 0,5 %. | |

2. Procédé d'électrodéposition d'un alliage d'or selon la revendication 1 ; ledit procédé comprenant l'utilisation d'une solution aqueuse comprenant un sel d'or (Au), un sel de fer (Fe) et un sel de vanadium (V), et éventuellement un ou plusieurs sels d'autres métaux avantageusement choisis parmi les sels de cobalt (Co), de palladium (Pd), de ruthénium (Ru), pour moduler les teintes de couleur finales ; et comprenant éventuellement en outre de faibles quantités d'un ou de plusieurs sels de tellure (Te), de gallium (Ga) ou de Bismuth (Bi), en tant qu'auxiliaires de brillance et d'affineurs de grain, dans lequel l'or en tant que métal est dans la plage comprise entre 0,5 et 3 g/l, dans lequel Fe et V en tant que métaux sont fournis en des concentrations dans la plage comprise entre 0,2 et 1 g/l, respectivement, et ayant un pH tamponné dans la plage comprise entre 7 et 10.

3. Procédé selon la revendication 2, dans lequel l'or en tant que métal est dans la plage comprise entre 0,7 et 1,8 g/l.

4. Procédé selon la revendication 2, dans lequel Fe et V en tant que métaux sont fournis en des concentrations de 0,6 g/l, respectivement.

5. Procédé selon la revendication 2, dans lequel Co, Pd et Ru, le cas échéant, sont chacun fournis en des concentrations dans la plage comprise entre 0,005 et 0,5 g/l, dans lequel les concentrations concernent le métal en solution.

6. Procédé selon la revendication 2, dans lequel Te, Ga, Bi ou des combinaisons de ceux-ci sont introduits dans la solution sous forme de sels solubles de ceux-ci ou de complexes stables de ceux-ci dans les conditions de travail de la solution, en des quantités pour chaque métal dans la plage comprise entre 0,005 et 0,015 g/l en tant que métal.

7. Procédé selon l'une quelconque des revendications 2 à 6, ayant un pH tamponné dans la plage comprise entre 7,5 et 9,5.

8. Procédé selon l'une quelconque des revendications 2 à 7, comprenant un ou plusieurs agents complexants en des concentrations dans la plage comprise entre 20 et 50 g/l.

9. Procédé selon l'une quelconque des revendications précédentes, dans lequel un tensioactif est fourni en des quantités d'au plus 1 g/l.

10. Solution aqueuse pour l'électrodéposition d'un alliage d'or selon la revendication 1 ; ladite solution comprenant un sel d'or (Au), un sel de fer (Fe) et un sel de vanadium (V), et éventuellement un ou plusieurs sels d'autres métaux avantageusement choisis parmi les sels de cobalt (Co), de palladium (Pd), de ruthénium (Ru), pour moduler les teintes de couleur finales ; et comprenant éventuellement en outre de faibles quantités d'un ou de plusieurs sels de tellure (Te), de gallium (Ga) ou de Bismuth (Bi), en tant qu'auxiliaires de brillance et d'affineurs de grain, dans lequel l'or en tant que métal est dans la plage comprise entre 0,5 et 3 g/l, dans lequel Fe et V en tant que métaux sont fournis en des concentrations dans la plage comprise entre 0,2 et 1 g/l, respectivement, et ayant un pH tamponné dans la plage comprise entre 7 et 10.
